

Patented Oct. 26, 1926.

1,604,544

# UNITED STATES PATENT OFFICE.

LUIGI ARNONE, OF FLORENCE, ITALY.

SPECIAL CARBON FOR THE STARTING OF A VOLTAIC ARC WITH ULTRA VIOLET RAYS.

No Drawing. Application filed November 14, 1923. Serial No. 674,714, and in Italy December 19, 1922.

The invention relates to an improved carbon for use in the artificial formation of special ultra-violet rays for heliotherapeutic purposes; such invention essentially comprises special homogeneous carbons, which, when applied to an appropriate lamp, yield the desired results.

The composition and the process for obtaining the special homogeneous carbons for the production of the ultra-violet rays are as follows.

For the manufacturing of the said homogeneous carbons, the Bremer system is generally followed. The constituents of the mixture are approximately as follows:

|                  | Parts.      |
|------------------|-------------|
| Aerated graphite | about 76.63 |
| Retort-carbon    | 5           |
| Lamp-black       | 1           |
| Vegetable carbon | 4           |

#### Metals and metalloids.

|                                            | Per cent. |
|--------------------------------------------|-----------|
| Calcium (Ca)                               | 5         |
| Magnesium (Mg)                             | 3         |
| Strontium (Sr)                             | 0.9       |
| Ferrum (Fe)                                | 0.9       |
| Rare earths                                | 0.97      |
| Fluor (Fl)                                 | 2.50      |
| Silica (SiO <sub>2</sub> )                 | 0.1       |
| Aluminium (Al), sodium (Na), potassium (K) | traces.   |

With the ordinary methods the pulverization and the perfect mixture of the component parts is obtained by shaking up the powders in a closed cylinder, and then adding as much benzole as is requisite for the formation of a thick paste; the paste being worked for hours with a reverse movement

40 of pasting machine. As soon as a homogeneous paste has thus been obtained, it is strained through a stout bronze cylinder (strainer) where it is compressed at about 200 atmospheres in a suitable hydraulic press.

45 The compressed paste is withdrawn from the holes in the form of a slender candle, of the thickness required for the arc, and is cut into lengths of about 25 cm.

The carbons thus formed are exposed to the air and well dried, after which they are ready for baking. This is the most delicate of operations, it being the one upon which the successful production of the carbons depends.

55 There are several kinds of ovens and

methods of baking; but for the purpose in question Hoffmann's oven is preferred, this oven being divided into 24 compartments wherein baking is effected, the passage from one compartment to another being effected every 24 hours.

As a source of heat it is convenient to use the Siemens's apparatus, which is a large gas producer. In spite of this improved method, however, continual superintendence and great experience are necessary.

Finally, the carbons are rubbed clean with a piece of linen cloth and soaked in gum arabic. This varnish encloses the carbon in a case or coating, and protects it against humidity. The carbons, thus varnished or coated, are exposed to the sun, or to the open air, for one day, at least; and after this treatment they remain smooth and glossy and may be handled without smudging the hands.

The apparatus for the obtainment of the ultra-violet rays produced by means of said carbons, must handle the carbons with ease, and in such manner as to ensure the desired location of the arc in relation to a suitable condenser and light-directing tube.

#### Claims.

1. Carbons for obtaining arc formation with ultra-violet rays for the purpose described, in which such carbons are essentially composed of the following constituents:

|                  | Parts. |
|------------------|--------|
| Aerated graphite | 76.63  |
| Retort-carbon    | 5      |
| Lamp-black       | 1      |
| Vegetable carbon | 4      |

#### Metals and metalloids.

|                                            | Per cent. |
|--------------------------------------------|-----------|
| Calcium (Ca)                               | 5         |
| Magnesium (Mg)                             | 3         |
| Strontium (Sr)                             | 0.9       |
| Ferrum (Fe)                                | 0.9       |
| Rare earths                                | 0.97      |
| Fluor (Fl)                                 | 2.50      |
| Silica (SiO <sub>2</sub> )                 | 0.1       |
| Aluminium (Al), sodium (Na), potassium (K) | traces.   |

2. A process for the production of carbons for the purpose described, in which the constituents set forth in claim 1 are reduced to a powder, are then mixed with benzol to form a paste, are then compressed and

strained, are then baked, then soaked in gum arabic and are finally dried by exposure to air.

3. A process for the production of carbons for the purpose described, in which the constituents set forth in claim 1 are reduced to a powder and mixed together, are then formed

into a paste, are then strained and subjected to high pressure to form carbons of candle form which are exposed to the air, are then baked and cleaned and are finally coated with gum and again exposed to the air. 10

PROF. LUIGI ARNONE. [L. S.]